

## UNITED STATES PATENT OFFICE

PAUL D. MERICA, OF WESTFIELD, AND JAMES S. VANICK, OF ELIZABETH, NEW JERSEY,  
ASSIGNORS, BY MESNE ASSIGNMENTS, TO THE INTERNATIONAL NICKEL COMPANY,  
INC., OF NEW YORK, N. Y., A CORPORATION OF DELAWARE

## ALLOY

No Drawing.

Application filed July 3, 1928. Serial No. 190,515.

Our invention relates to alloys and particularly to cast iron alloys adapted to resist corrosion or oxidation. We have discovered that if nickel, copper and chromium be added as alloying ingredients to cast iron, particularly within the proportions hereinafter recited, an alloy is produced which can be cast and handled in the foundry in substantially the same way as ordinary gray cast iron. In 10 making the alloy we add to cast iron having the usual carbon content of cast iron, namely from about 2% to 4% of carbon, nickel, copper and chromium. The nickel and copper is preferably added as an alloy in amount from 15 about 5% up to about 50%, the ratio of nickel to copper in said alloy being preferably in the neighborhood of 2.2%. The chromium is added preferably from 1/2% up to 15% and the added alloying metals also preferably contain from 1.5 to 4% of carbon and from 1/2% to 3% of silicon.

For example, good results are obtained with a cast iron alloy containing 20% of the alloy known as Monel metal (in which 25 the ratio of nickel to copper is 2.2), 2% of chromium, 3% of carbon and 2% of silicon. The preferred range of alloy is as follows:

Nickel 10-20%, copper 2-10% (or copper greater than 2% but less than 1/2 of the nickel 30 content), carbon 2-3.5%, silicon 0.25-2.5%, chromium up to 5%, manganese and other elements as usual for cast iron.

The alloy may be cast in sand molds to form a gray cast iron casting, or it may be cast 35 against a chill to form white iron. The shrinkage of such castings is about the same as that of ordinary cast iron. When cast under the ordinary conditions of making gray cast iron castings, the carbon is partly in the 40 graphitic state so that the castings are gray and readily machinable. Such castings have a transverse strength comparable with that of an ordinary 2% silicon gray iron casting. Thus, test bars show 130 Brinell test and 45 3000 lbs. in transverse strength.

Castings thus made are, however, greatly superior to ordinary cast iron in corrosion 50 resistant properties and are comparable in this respect with Monel metal castings or the ordinary cast brasses or bronzes. Thus,

when our casting is subjected to 5% sulphuric acid aerated at ordinary temperatures, the corrosion is about at the rate of 350 milligrams per square decimeter per day. This is about the same as that of lead, bronze or 55 Monel metal while plain cast iron shows about 30,000 milligrams per square decimeter per day.

When our preferred alloy is subjected to aerated 3% sodium chloride solution it shows 60 a loss of 50 milligrams per square decimeter per day as compared to 300 for ordinary cast iron. Such an alloy will only rust superficially and appears to be quite stable toward ordinary atmospheric and other corroding influences such as are ordinarily encountered in industrial practice. The castings are also amenable to heat treatment to render them within suitable composition limits either soft or hard, with corresponding variations in malleability and toughness.

The alloys are particularly adapted for castings of either the gray iron or chilled iron type where anti-corrosive material is needed such for example as in valves, chemical apparatus, etc. Among other characteristic advantages of our alloy, particularly within the preferred range, are the following:—the alloy is substantially non-magnetic at ordinary and at high temperatures; 75 it has a high electrical resistance which is especially useful in the absence of magnetism; it has a high coefficient of thermal expansion from room temperature up to about 300° C., which is approximately .000018 per degree centigrade; it is moderately heat resistant, that is, relatively stable at higher temperatures up to about 1500° F., at the same time being substantially free from the phenomenon of “growth”.

It can be readily welded by the usual autogenous methods and is more satisfactory than iron for this purpose as it is not thereby hardened in the weld area as is ordinary cast iron. The above properties 95 make the alloy valuable for many purposes, such as castings subjected to high temperatures where scaling should be kept at a minimum and volume stability is important. It is valuable for electrical castings especially 100

where the absence of magnetism is important, and its high coefficient of thermal expansion fits it for mechanical construction where it is to be associated with other high expansion metals or alloys, such as aluminum, brass or similar alloys.

Other ingredients may be added such as aluminum and manganese. The manganese may be from .3 to 10% and the aluminum from nothing up to about 3%.

While we have described a preferred proportion of our invention it will be understood that the invention is not limited thereto but may be varied within the scope of the following claims.

We claim:

1. An alloyed cast iron containing more than 50% of iron having from 2% and up to about 4% carbon, and also containing nickel, 20 copper and chromium, the nickel being from 10-20%, the copper being over 1% but less than  $\frac{3}{4}$  of the nickel and the chromium from a material percentage to not over 10%.

2. An alloy cast iron containing more than about 50% of iron, carbon from about 2% to about 3.5%, nickel about 10% to about 20%, copper about 2% to about 10%, chromium from a material percentage up to about 5% and silicon from about 0.25% to about 3.0%.

3. An alloy cast iron as set forth in claim 2, in which the nickel is present to an extent of approximately twice the copper content.

35. In testimony whereof we have hereunto set our hands.

PAUL D. MERICA.  
JAMES S. VANICK.

40

45

50

55

60

65